

A. DEAN.

## Process of and Machinery for Making Paper Pulp from Wood.

No. 241,311.

Patented May 10, 1881.



**WITNESSES:**

George Cole Madden  
James T. Goodfellow

**INVENTOR:**

Alexander Dean

A. DEAN.

# Process of and Machinery for Making Paper Pulp from Wood.

No. 241,311.

Patented May 10, 1881.

FIG. 6.



FIG. 2.



**WITNESSES:**

*INVENTOR:*

George Cole Madden  
James T. Goodfellow

Alexander Dean

A. DEAN  
Process of and Machinery for Making Paper Pulp  
from Wood.

No. 241,311.

Patented May 10, 1881.

FIG. 8.



FIG. 9.



WITNESSES:

George Cole Madden  
James T. Goodfellow.

INVENTOR:

Alexander Dean

# UNITED STATES PATENT OFFICE.

ALEXANDER DEAN, OF LUZERNE, NEW YORK.

## PROCESS OF AND MACHINERY FOR MAKING PAPER-PULP FROM WOOD.

SPECIFICATION forming part of Letters Patent No. 241,311, dated May 10, 1881.

Application filed January 24, 1880.

*To all whom it may concern:*

Be it known that I, ALEXANDER DEAN, of Luzerne, in the county of Warren and State of New York, have invented certain new and useful Improvements in the Process of and Machinery for Making Paper-Pulp from Wood, of which the following is a specification.

My invention relates to certain improvements in mechanical devices and combinations of contrivances and processes for transforming sticks of wood into fine pulpy fibers suitable to be used as a large constituent of printing and other fine papers.

The principal objects of my improvements are to provide superior devices and processes for cutting sticks of wood into small pieces of suitable grain-length, for disintegrating the pieces of wood and softening and separating the fibers thereof, for reducing the fibers in water, and for separating the fine fibers in water from the coarse fibers and particles.

In my new process for transforming sticks of wood into fine fibers in water the sticks are first cut into suitable small pieces, chips, or bits of proper grain-length, and such pieces, chips, or bits of wood are disintegrated, softened, and divided into fibers in water by subjecting the same with water to the whirling and rending action of a common Jordan engine, with or without first subjecting the pieces, chips, or bits of wood, without water, to the action of a disintegrating-mill; and the fibers in water are reduced to fine pulpy fibers by subjecting them with water to the grinding action of millstones, with or without first subjecting them in water to the beating, brushing, and soft rubbing action of a common pulping-engine.

The machinery which is useful in carrying out my new process for preparing fine fibers in water from sticks of wood, and which embraces the mechanical parts of my invention, is illustrated in the accompanying drawings, in which—

Figure 1 is a plan of the whole machinery. Fig. 2 is an elevation of a section of the wood-cutting device, the section of the rotary cutter being at the line  $z z$  in Fig. 1, and of the stationary part at the line  $y y$  in the same figure. Fig. 3 is a side elevation of the rotary cutter. Figs. 4 and 5 are side and edge elevations of a stick of wood, showing at one end about the

shape of the cuts made by the cutting device. Fig. 6 is an elevation of the same machinery, seen in the direction pointed by the arrow  $x$  in Figs. 1, 7, and 8, some parts being shown in section. Fig. 7 is an elevation of the same, viewed in the direction indicated by the arrow  $w$  in Figs. 1, 6, and 9, a part being in section. Fig. 8 is an elevation of the same, seen in the direction pointed by the arrow  $v$  in Figs. 1, 6, and 9, some portions being in section. Fig. 9 is an elevation of the same, viewed in the direction indicated by the arrow  $u$  in Figs. 1, 7, and 8. 65

Like letters refer to like parts in the several figures.

A is the stationary support of the apparatus. B, Fig. 3, is a rotary cutter in the form of two conic frustums united at their small ends and fastened axially upon a shaft, V, and furnished with suitably projecting blades or teeth  $b$  on the two oppositely-inclined conic portions, for cutting thin pieces, chips, or bits of wood of suitable grain-length for paper-pulp from sticks Z, properly presented endwise thereto by the inclined stationary wood-feeder C, Figs. 1 and 2, which is in the form of an open-ended box conformed to and extending at one end, c, into the angle of the cutter. This combination of the reversely conical inwardly-inclined rotary cutter B and the inclined wood-feeding support C, conformed to and extending into the angle of the rotary cutter, constitutes a very simple and superior device or engine for reducing sticks of wood of the ordinary shapes split from logs into thin pieces, chips, or bits preparatory to being made into paper-pulp. This superiority results mainly from the fact that a stick of wood placed endwise in the feeder C is fed by its gravity to the rotary cutter B, which, as it revolves, continually forces the contiguous end of the stick into the angle formed by the junction of the two conical cutting portions, which cut thin pieces, 75 chips, or bits from two opposite sides of the stick in directions inclined to each other and to the length and width of the stick and of its fibers, about as indicated at  $t$  in Figs. 4 and 5, until the whole stick is thus cut away to a small bit at its other end, and from the fact that the chips, pieces, or bits thus cut obliquely from opposite sides of the stick have their fibers inclined or oblique to the cut surfaces 80 85 90 95 100

thereof, so that the fibers of such pieces, chips, or bits are pointed or beveled at their ends, and are very easily separable, and are of much greater length than in bits, chips, or pieces of 5 the same thickness cut from like sticks of wood in directions perpendicular, or nearly so, to the lengthwise direction of the fibers.

D, Fig. 7, is an upright tapering rubber, secured to and revolved by and with a rotary 10 shaft, d, and having its outer surface formed with longitudinal flutes, ribs, or grooves e; and E is a stationary casing surrounding the rubber D, and having its inner surface formed with ribs, flutes, or grooves corresponding to those 15 of the adjacent opposite surface of the rotary rubber. These ribs, flutes, or grooves are essentially like those in the mills that are commonly used for grinding bark in tanneries, and a good common bark-grinding mill is a good 20 substitute or equivalent for the mill composed of the rotary part D and its stationary casing E.

F is an inclined chute extending from the bottom of the cutting-engine B C to the top of the mill D E, so that the pieces, chips, or bits 25 of wood cut from sticks by the cutting-engine will be automatically fed from the cutting-engine into the disintegrating-mill by said chute. The pieces, chips, or bits of wood are thus passed dry, or without water, through that mill, 30 which will rub and disintegrate them into smaller pieces, bits, or particles.

G, Fig. 6, is the rotary tapering bladed cylinder, and H is the corresponding bladed stationary casing, of a common Jordan engine for 35 grinding paper-pulp.

I is an inclined chute, by which the disintegrated pieces and bits of wood discharged from the bottom of the mill D E are automatically conducted from the latter into the Jordan engine. 40

J is a pipe for supplying a suitable stream of water to the Jordan engine with the stream of small pieces or bits of wood conducted thereto by the chute I.

K is the tank or reservoir of a common stuff-chest, having therein a rotary stirrer, L, as usual in paper-mills; and f is a pipe for conducting into the stuff-chest the fibers of wood in water discharged by the Jordan engine. 45

M, Fig. 1, is the circuit-tank, and N is the beating-roll, of a common pulping-engine, furnished with a bed of knives conformed to the bladed roll N, and between adjacent inclines g g', as usual in such engines. Water can be 50 supplied to the tank M by a pipe, h, or otherwise.

O is a rotary pump, of any suitable known construction, connected by a conduit, i, Fig. 6, with the stuff-chest K, and having a discharge-pipe, i', leading to the tank M, so that by the operation of the pump the fibers of wood in water will be transferred from the stuff-chest into the pulping-engine. 60

The pump O can be dispensed with by having the pulping-engine M N lower than the stuff-chest K, and connected therewith by a gated trough or pipe, through which the con-

tents of the stuff-chest can run by gravity into the pulping-engine; or the fibers in water can be discharged from the Jordan engine directly 70 into the pulping-engine by means of a direct pipe or hose connection, as indicated by dotted lines at f' in Fig. 6; but I commonly prefer to discharge the fibers in water from the Jordan engine into the stuff-chest, and to thence 75 transfer the same into the pulping-engine M N, or into two or more such pulping-engines, as may be required, to reduce all the fibers in water discharged by the Jordan engine.

P P', Fig. 8, are a pair of millstones, which 80 are preferably of the quality of common grindstones, instead of the ordinary harder burr-stones, and are mounted and dressed essentially like common millstones for grinding grain, and have an inlet-passage, j, and outer 85 casing, j', with an annular outlet and trough-like conduit, j".

Q is a pipe by which the woody fibers suspended in water can be fed from the tank M into the millstones; but any other suitable 90 known means can be used for feeding the fibers in water from the tank M into each of the one, two, or more pairs of such millstones as shall be required to properly grind all the fibers in water from the Jordan engine, pulping-engine, 95 or pulping-engines that shall be used.

R, Figs. 1, 7, and 9, is a wire-cloth screen in the form of a turning endless apron, having thereon side guards, k, and supported by drums l l' and a roller, l", and of proper fineness to let 100 the sufficiently fine fibers in water pass through the screen and prevent the passage there-through of larger fibers and particles.

S is a trough or chute for conducting the fibers in water from the millstones P P' onto 105 the upper stretch of the screen R; and T is a trough arranged between the upper and lower stretches of the screen, to receive and conduct off the fine fibers in water that shall pass through the upper stretch of the screen. 110

U, Figs. 8 and 9, is a pipe arranged across and between the upper and lower stretches of the screen R, and in communication with a supply of water, and having in its lower side a slot or series of small holes, through which the 115 water will forcibly rush against the upper surface of the lower stretch of the screen, so as to thereby pass through the screen and progressively remove therefrom the coarse fibers and particles that shall be progressively separated 120 by the upper stretch of the screen from the fine fibers in water.

When desired, the fibers in water can be conducted onto the upper stretch of the screen R by a suitable pipe or hose extending thereto 125 from the tank M of the pulping-engine, as indicated by dotted lines at Y in Fig. 7, or from the discharge-pipe i' of the pump O, as represented by dotted lines at W in Fig. 1, or from the discharge-pipe f of the Jordan engine, as indicated by dotted lines at X in Fig. 7. 130

When practicable in carrying out this invention, I commonly prefer that the first reducing device used shall be highest in position, and

each succeeding device used lower than the preceding one, and the several devices connected in succession by inclined passages or chutes, through which the materials shall be transferred by their gravity from the preceding reducing device into the next one. However, in carrying out my improvements in making fine screened pulpy fibers in water from sticks of wood, and in machinery therefor, the several 5 reducing devices can be in any suitable relative positions, and any suitable known means can be employed or combined with the reducing devices for actuating the same from any suitable known motor or motors, and for transferring the materials acted upon from any one 10 of the reducing devices to the next one used.

In the drawings, V is a rotary shaft which supports and revolves the cutter B, and from which shaft rotary motion is imparted to the 20 rubber D by the gears  $m$   $m'$  and shaft  $d$ , Fig. 7; to the rotary part G, Fig. 6, of the Jordan engine by the pulley  $n$ , belt  $n'$ , pulley  $n^2$ , and shaft  $n^3$ ; to the stirrer L in the stuff-chest by the gears  $m$   $m'$ , shaft  $d$ , Fig. 7, pulley  $o$ , belt 25  $o'$ , and pulley  $o^2$ ; to the rotary pump O by the pulley  $p$ , belt  $p'$ , and pulley  $p^2$ ; to the beating-roll N of the pulping-engine by the pulley  $q$ , belt  $q'$ , pulley  $q^2$ , and shaft  $q^3$ ; to the upper millstone, P, by the gears  $m$   $m'$ , shaft  $d$ , Fig. 7, 30 pulley  $r$ , belt  $r'$ , pulley  $r^2$ , and shaft  $r^3$ , and to the endless apron-screen R by the gears  $m$   $m'$ , shaft  $d$ , gears  $s$   $s'$ , shaft  $s^2$ , pulley  $s^3$ , Fig. 1, belt  $s^4$ , and pulley  $s^5$ , fast on the shaft of the drum  $l$ .

35 The operation of the apparatus represented by full lines in the drawings in transforming sticks of wood into fine screened pulpy fibers in water is as follows: The sticks, Z, of wood, of any suitable shape, placed endwise in the 40 feeder C of the cutting-engine, will be thereby cut into small thin pieces, chips, or bits, which will have the fibers oblique therein, and of suitable grain-length for making into pulp, and which will pass through the chute F into the 45 rubbing-mill D E without water, and will be disintegrated by that mill and discharged through the chute I into the Jordan engine G H, with water from the pipe J. The Jordan engine will rub and rend the disintegrated 50 wood and separate the fibers thereof more or less finely in the water, according to the closeness with which the part G is adjusted in the casing H and to the back-pressure therein, and will discharge the fibers with the water, by 55 the pipe f, into the stuff-chest K, in which the fibers will be kept suspended in water by the stirrer L, while the rotary pump O shall be made to transfer the fibers in water, through the passages  $i$   $i'$  from the stuff-chest, into the 60 circuit-vat M of the pulping-engine, either constantly or intermittently, as shall be required. The pulping-engine M N beats, brushes, and smoothly rubs the fibers in water, and thereby renders them very soft and thin in diameter; 65 and the conduit Q is made to feed the soft fibers in water, as required, from the tank M into the millstones P P', through which the

fibers in water are passed, and thereby ground finer, and are conducted therefrom by the trough S onto the turning endless apron-screen 70 R, through the upper stretch of which the soft fine portion of the fibers pass with the water, and are conducted off by the trough T, to be separated from the water, while the larger fibers and particles that are stopped by the 75 screen are progressively removed from the latter by water discharged by the pipe U.

It will be observed that in the apparatus illustrated in the drawings the parts D E and chutes F I serve to conduct the small pieces, 80 chips, or bits of wood from the cutting-engine B C to the Jordan engine G H, whether the pieces, chips, or bits shall or shall not be disintegrated by the parts D E, and that when the part D shall be set or adjusted endwise so 85 loosely in the shell E, or shall be removed therefrom so far as to not reduce the passing pieces, chips, or bits of wood, the parts D and E will then serve merely as a part of the means for transferring the pieces, chips, or bits from 90 the cutting-engine into the Jordan engine, and the Jordan engine will then act in immediate succession and combination with the cutting-engine, the same as if the chips or pieces of wood were passed from the cutting-engine into 95 the Jordan engine through a chute extending from the bottom of the cutting-engine B C directly to the inlet of the Jordan engine, as indicated by the dotted lines at F' in Fig. 6.

This direct combination of the cutting-engine B C, Jordan engine G H, means for transferring the pieces, chips, or bits of wood from the cutting-engine into the Jordan engine, and mechanism for simultaneously actuating the Jordan engine and cutting-engine constitutes 100 105 an effective automatic apparatus, which I commonly use, and sometimes prefer, for transforming sticks of tender wood into coarse fibers in water.

In order, however, to more thoroughly reduce a greater quantity of the same size and quality of pieces or chips of wood to fibers in water in a given time, I commonly prefer to use the parts D and E without water as a reducing-mill, and have them adjusted so closely 110 together that they will finely rub and disintegrate the chips or pieces of wood before the latter shall be passed into the Jordan engine.

It will also be observed that in the apparatus represented by the drawings the pipe f, 120 stuff-chest K L, pump O, pipes  $i$   $i'$ , pulping-engine M N, and pipe Q will serve to transfer the fibers in water from the Jordan engine G H to the millstones P P', whether the roll N of the pulping-engine shall or shall not operate 125 to reduce the fibers in such transfer, and that when the roll N shall not operate to reduce the fibers the pulping engine then will serve merely as a stuff-chest part of the means for transferring the fibers in water from the Jordan engine into the millstones P P', and that the millstones will then operate in immediate combination with the Jordan engine substantially the same as when the fibers in water are 130

conducted from the Jordan engine into the millstones by a direct pipe or hose, as indicated by dotted lines at  $f^2$  in Figs. 1 and 6, and the same as when the fibers in water are 5 discharged by the Jordan engine through the pipe  $f$  into the stuff-chest K, and are fed from the latter into the millstones by the conduit  $i$ , pump O, and a pipe or hose leading from the pump directly into the millstones, as indicated 10 by the dotted lines at  $i^2$  in Figs. 1 and 6, and as I generally prefer in combining and using one, two, or more pairs of millstones directly with the Jordan engine.

This direct use and combination of a Jordan engine, millstones, and means for actuating the millstones and Jordan engine, and for transferring the fibers in water from the Jordan engine through a stuff-chest to the millstones, has proved in practice to be a very effective apparatus, which I generally prefer for reducing suitable small pieces, chips, or bits of wood into fine paper-pulp fibers.

However, when the fibers require to be more thoroughly softened and fibrilized I sometimes prefer to subject them in water to the beating, brushing, and soft rubbing action of the pulping-engine before subjecting them in water to the grinding action of the millstones.

The process for transforming sticks of wood 30 into fibers in water by first cutting the sticks into pieces or bits of suitable grain-length, and then subjecting them with water to the rending action of the Jordan engine, and the process for converting pieces or bits of wood of 35 suitable grain-length into fine fibers by subjecting the pieces or bits of wood with water to the action of the Jordan engine, and then reducing the fibers by subjecting them in water to the grinding action of millstones, are sub- 40 processes embraced in my above-described process for transforming sticks of wood into fine fibers in water by first cutting the sticks into pieces or bits of suitable grain-length, then softening the pieces or bits and separating the 45 fibers thereof by subjecting the same with water to the action of the Jordan engine, and finally reducing the fibers by subjecting them in water to the grinding action of millstones.

By the introduction of my above-described 50 improvements in the latter process it becomes my improved process for transforming sticks of wood into fine fibers in water, by first cutting the sticks into pieces of suitable grain-length, next disintegrating the pieces by subjecting them without water to the reducing action 55 of the rubbing-mill, then softening the disintegrated pieces or bits of wood and separating the fibers thereof by subjecting the same with water to the whirling and rending action 60 of the Jordan engine, next fibrilizing, pulping, and reducing the fibers by subjecting them in water to the beating, brushing, and soft rubbing action of the pulping-engine, and finally reducing the pulpy fibers by subjecting them 65 in water to the grinding action of millstones.

This improved process embraces several combinations of steps or sub-processes which are

of much practical importance and yield distinct results subsidiary to the main one, to wit: the improved sub-process of converting 70 small pieces of wood into fibers in water by first disintegrating the pieces by subjecting them without water to the action of the reducing-mill, and next softening the disintegrated wood and separating the fibers thereof by 75 subjecting the same with water to the soft rendering action of the Jordan engine; also, the sub-process of converting disintegrated pieces or bits of wood into soft pulpy fibers by first softening the disintegrated pieces or bits of 80 wood and separating the fibers thereof by subjecting the same with water to the fine rendering action of the Jordan engine, and then softening and reducing the fibers by subjecting them in water to the beating, brushing, and 85 smooth rubbing action of the pulping-engine; also, other combinations of steps or sub-processes hereinafter claimed as of my invention.

Prior to my invention pulp had sometimes been made from blocks of wood by pressing 90 the latter against a revolving grindstone supplied with water, whereby the wood was reduced to a mixture in water of useful fibers and useless fine dust, slivers, and bits of greatly different sizes, and then screening such mixture and passing the useful screened portion thereof in water through millstones. In that process a large percentage of useless waste, in the form of fine dust and coarse slivers and bits, was the result of the abrading action of 100 the grindstone against the blocks of wood, and the grindstone was the only mechanical disintegrator used in reducing the wood from its condition in blocks to that of which a screened portion in water was passed through the millstones. I avoid that waste of stock by my invention, which differs essentially from that prior process, because according to my invention the fibers are not ground or abraded from blocks or sticks of wood by pressing the latter 110 against a grindstone or other similar grinding or abrading surface supplied with water; and, according to my herein-described invention for reducing sticks of wood into pulp, the sticks must be first cut or reduced into chips, small 115 pieces, or bits, which must be passed with water through the well-known Jordan engine before being subjected in water to the action of millstones or other pulp-producing mechanism.

I believe that sometimes, in reducing sticks 120 of wood into pulp, the sticks have been held by hand against a rest, and thereby presented to the upright face of a rotary cutter-wheel, which cut the wood into chips of definite grain-length, and received the chips inside and delivered them into an upright crushing-mill, by which the chips were split and broken into small pieces or bits, which were afterward subjected in water to the action of the beating roll and bed of a common or improved pulping-engine. Therefore I do not herein broadly claim reducing sticks of wood to small pieces or bits of suitable grain-length for making into pulp by first cutting the sticks into suitable

chips and then splitting and breaking the chips into small pieces or bits by passing the chips through a crushing-mill; and do I broadly claim the combination of a rotary cutter and rest for cutting sticks of wood into chips of definite grain-length with an upright crushing-mill for disintegrating the chips and means for operating the crushing-mill and cutter and for delivering the chips from the cutter into the crushing-mill.

Still, my improved self-feeding cutting device, composed of the double cones B, with cutters b, and the inclined feed-box C, shaped and arranged as herein described and shown, is essentially different from and far superior to the hand-fed chip-receiving cutter-wheel and rest above mentioned for cutting sticks of wood into suitable chips for making into pulp; and my herein-described combination of the cutting device B b C with the reducing-mill D E constitutes an improved mechanism for reducing sticks of wood into small pieces or bits suitable for making into pulp.

Furthermore, I do not herein broadly claim the process of reducing chips of wood to pulp by subjecting them first to the action of a crushing-mill, and afterward in water to the action of a pulping-engine; nor do I claim the combination of a crushing-mill, pulping-engine, and means for operating the pulping-engine and crushing-mill, and for transferring small bits of wood from the crushing-mill into the pulping-engine. In my present invention for reducing chips or bits of wood into pulp or fibers in water it is essential that the chips or bits of wood shall be passed with water through and subjected to the peculiar well-known reducing action of the Jordan engine, which latter is an essential element of each combination of parts which I use and hereinafter claim for reducing chips or bits of wood into pulp or fibers in water.

Sometimes sticks of wood have been cut or sawed and crushed into pieces, which were passed through a picking or breaking mill and thereby reduced into bits, which were passed with water through millstones, and thereby ground, and I do not herein claim that process of reducing sticks of wood into pulp or fibers in water; nor do I claim, broadly, the combination of a rotary cutting device, picking or breaking mill, and millstones.

It is essential to that part of my invention in which millstones are used that the chips or bits of wood, before being passed through the millstones, shall be subjected with water to the peculiar rapid brushing and reducing action of the Jordan engine, by which larger chips or bits of wood can be received and reduced in water into fibers of very uniform size, and with far greater rapidity and less expense than by the use of millstones alone.

The Jordan engine has been heretofore often used in preparing or finishing paper-pulp; but I am not aware that before my invention a Jordan engine had been used in connection with a mill or mechanism which cut, sawed, or re-

duced sticks or pieces of wood into small chips or bits, which were passed with water through the Jordan engine; and I do not know nor believe that prior to my invention a Jordan engine was used to reduce chips or bits of wood into fibers, which were afterward passed with water through millstones or subjected to the action of a common pulping-engine.

70

75

What I claim as my invention is—

1. The process of making fine pulpy fibers from sticks of wood by first cutting the sticks into small pieces, chips, or bits of suitable grain-length, subsequently softening the pieces, 80 chips, or bits and separating the fibers thereof by subjecting the same with water to the whirling and fine-rending action of a Jordan engine, and finally reducing the fibers by subjecting them in water to the grinding action of 85 millstones, all substantially as described.

2. The sub-process of transforming sticks of wood into fibers in water by first cutting the sticks into pieces, chips, or bits of suitable grain-length, and afterward softening the pieces, 90 chips, or bits and separating the fibers thereof by subjecting the same with water to the rending action of a Jordan engine, all as described.

3. The sub-process of converting small pieces, 95 chips, or bits of wood into fine fibers in water by first softening the pieces, chips, or bits, and separating the fibers thereof by subjecting the same with water to the fine-rending action of a Jordan engine, and finally reducing the fibers 100 by subjecting them in water to the grinding action of millstones, all substantially as described.

4. The improved sub-process of converting suitable pieces of wood into fibers in water by 105 first disintegrating the pieces by subjecting them without water to the reducing action of a rubbing-mill, as described, and then softening the disintegrated pieces and separating the fibers thereof by subjecting the same with water to the fine-rending action of a Jordan engine, as set forth.

5. The improved sub-process of transforming sticks of wood into fibers in water by first cutting the sticks into pieces of suitable grain-length, next disintegrating the pieces by subjecting them without water to the dry-rending action of a reducing-mill, and then softening the disintegrated wood and separating the fibers thereof by subjecting the same with water to 120 the fine-rending action of a Jordan engine, all substantially as described.

6. The improved sub-process of converting pieces of wood into fine fibers in water by first disintegrating the pieces by subjecting them 125 without water to the rending action of a reducing-mill, next softening the disintegrated wood and separating the fibers thereof by subjecting the same with water to the fine-rending action of a Jordan engine, and finally reducing the 130 fibers by subjecting them in water to the grinding action of millstones, all substantially as set forth.

7. The improved process of transforming

- sticks of wood into fine pulpy fibers in water by first cutting the sticks into suitable pieces, next disintegrating the pieces by subjecting them without water to the dry reducing action of a rubbing-mill, then softening the disintegrated wood and separating the fibers thereof by subjecting the same with water to the fine-rending action of a Jordan engine, and finally reducing the fibers by subjecting them in water to the soft grinding action of millstones, all substantially as described.
8. The improved sub-process of converting small pieces or bits of wood into pulpy fibers in water by first softening the pieces or bits and separating the fibers thereof by subjecting the same with water to the fine-rending action of a Jordan engine, and then fibrilizing and pulping the fibers by subjecting them in water to the beating, brushing, and soft rubbing action of a pulping-engine, all as set forth.
9. The improved sub-process of converting small pieces or bits of wood into fine pulpy fibers in water by first softening the pieces or bits and separating the fibers thereof by subjecting the same with water to the fine-rending action of a Jordan engine, and then pulping and reducing the fibers by subjecting them in water first to the beating, brushing, and soft rubbing action of a pulping-engine, and next to the grinding action of millstones, all substantially as described.
10. The improved sub-process of converting pieces of wood into fibers in water by first disintegrating the pieces by subjecting them without water to the dry-rubbing action of a reducing-mill, as described, and then softening, separating, and reducing the fibers of the disintegrated wood by subjecting the latter in water first to the fine-rending action of a Jordan engine, and next to the beating, brushing, and rubbing action of a pulping-engine, as set forth.
11. The improved sub-process of converting sticks of wood into fibers in water by first cutting the sticks into pieces of suitable grain-length, and disintegrating the pieces by subjecting them without water to the dry-rending action of a rubbing mill, as described, and then softening, separating, and reducing the fibers of the disintegrated wood by subjecting the latter in water first to the fine-rending action of a Jordan engine, and next to the beating, brushing, and rubbing action of a pulping-engine, as set forth.
12. The improved sub-process of converting pieces of wood into fine pulpy fibers in water by first disintegrating the pieces by subjecting them without water to the dry-rending action of a reducing-mill, as described, and then softening, separating, and reducing the fibers of the disintegrated wood by subjecting the latter in water first to the fine-rending action of a Jordan engine, next to the beating, brushing, and soft rubbing action of a pulping-engine, and then to the grinding action of millstones, all as set forth.

13. The improved process of transforming sticks of wood into fine pulpy fibers in water by first cutting the sticks into pieces and disintegrating the latter by subjecting them without water to the dry-rending action of a rubbing-mill, next softening and separating the fibers of the disintegrated wood by subjecting the latter in water to the fine-rending action of a Jordan engine, and then softening and reducing the fibers by subjecting them in water first to the beating, brushing, and rubbing action of a pulping-engine, and then to the grinding action of millstones, all substantially as described.
14. The improved cutting device or engine having the rotary cutter B, in the form of two conic frustums united at their small ends, and furnished with blades or teeth b, in combination with the wood-feeding support C, inclined and fitting into the angle of the rotary cutter, substantially as described.
15. The combination of the cutting-engine B C, Jordan engine G H, means, substantially as described, for feeding pieces, chips, or bits of wood from the cutting-engine into the Jordan engine with water, and mechanism for actuating the Jordan engine and cutting-engine, substantially as set forth.
16. The combination of the Jordan engine G H, millstones P P', means, substantially as described, for transferring the fibers in water from the Jordan engine into the millstones, and mechanism for actuating the millstones and Jordan engine, substantially as set forth.
17. The combination of the cutting-engine, Jordan engine, millstones, means, substantially as described, for feeding the cuttings of wood from the cutting-engine into the Jordan engine with water, and for transferring the fibers in water from the Jordan engine into the millstones, and mechanism for actuating the millstones, Jordan engine, and cutting-engine, substantially as set forth.
18. The combination of the rotary cutter B, in the form of two conic frustums united at their small ends, inclined wood-feeder C, conformed to the rotary cutter, disintegrating-mill D E, means, substantially as described, for feeding the cuttings of wood from the rotary cutter into the disintegrating-mill, and mechanism for actuating said mill and rotary cutter, substantially as set forth.
19. The combination of the disintegrating-mill D E, Jordan engine G H, means, substantially as described, for feeding the disintegrated wood from said mill into the Jordan engine with water, and mechanism for actuating the Jordan engine and disintegrating-mill, substantially as set forth.
20. The combination of the cutting-engine, disintegrating-mill, Jordan engine, means, substantially as described, for feeding cuttings of wood from the cutting-engine into the disintegrating-mill and for feeding the disintegrated wood from the latter mill into the Jordan engine with water, and mechanism for actuating

the Jordan engine, disintegrating-mill, and cutting-engine, substantially as set forth.

21. The combination of the disintegrating-mill, Jordan engine, millstones, means, substantially as described, for feeding disintegrated wood from the mill into the Jordan engine with water, and for transferring the fibers in water from the Jordan engine into the millstones, and mechanism for actuating the millstones, Jordan engine, and disintegrating-mill, substantially as set forth.

22. The combination of the cutting-engine, disintegrating-mill, Jordan engine, millstones, means, substantially as described, for transferring the materials from the cutting-engine into the disintegrating-mill, and thence into the Jordan engine with water, and thence in water into the millstones, and mechanism for actuating the millstones, Jordan engine, disintegrating-mill, and cutting-engine, substantially as set forth.

23. The combination of the Jordan engine, pulping-engine, means, substantially as described, for transferring the fibers in water from the Jordan engine into the pulping-engine, and mechanism for actuating the pulping-engine and Jordan engine, substantially as set forth.

24. The combination of the Jordan engine, pulping-engine, millstones, means, substantially as described, for transferring the fibers in water from the Jordan engine into the pulping-engine, and thence into the millstones, and mechanism for actuating the millstones, pulping-engine, and Jordan engine, substantially as set forth.

25. The combination of the disintegrating-mill, Jordan engine, pulping-engine, means, substantially as described, for feeding the bits of wood from the disintegrating-mill into the Jordan engine with water, and for transferring the fibers in water from the Jordan engine into the pulping-engine, and mechanism for actuating the pulping-engine, Jordan engine, and disintegrating-mill, substantially as set forth.

26. The combination of the cutting-engine, disintegrating-mill, Jordan engine, pulping-engine, means, substantially as described, for transferring the woody material from the cutting-engine into the disintegrating-mill, thence

into the Jordan engine with water, and thence in water into the pulping-engine, and mechanism for actuating the pulping-engine, Jordan engine, disintegrating-mill, and cutting-engine, substantially as set forth.

55

27. The combination of the disintegrating-mill, Jordan engine, pulping-engine, millstones, means, substantially as described, for transferring the material from the disintegrating-mill into the Jordan engine with water, thence in water into the pulping-engine, and from the latter into the millstones, and mechanism for actuating the millstones, pulping-engine, Jordan engine, and disintegrating-mill, substantially as set forth.

65

28. The combination of the cutting-engine, disintegrating-mill, Jordan engine, pulping-engine, millstones, means, substantially as described, for transferring the material from the cutting-engine into the disintegrating-mill, thence into the Jordan engine with water, thence in water into the pulping-engine, and from the latter into the millstones, and mechanism for actuating the millstones, pulping-engine, Jordan engine, disintegrating-mill, and cutting-engine, substantially as set forth.

75

29. The combination of the prostrate turning endless apron-screen R, pulp-applying chute S, pulp-receiving trough T, and screen-washing pipe U, all arranged together for conjoint operation, as set forth.

80

30. The described combination of the endless apron-screen R, machinery for producing fine fibers in water from wood, mechanism for actuating the endless apron-screen and machinery for producing the fine fibers in water, means for progressively conducting the fibers in water from the machinery for producing the same onto the endless apron-screen and away from the latter, and means for progressively removing coarse fibers and particles from the screen by water, all the parts being substantially as described.

85

In testimony whereof I hereunto set my hand, in the presence of two subscribing witnesses, this 19th day of January, 1880.

ALEXANDER DEAN.

Witnesses:

WALTER SCOTT PORTEOUS,  
ANDREW PORTEOUS.